# EUROPEAN PATENT SPECIFICATION

(11) **EP 2 396 441 B1**
(45) Date of publication and mention of the grant of the patent: **05.12.2012**
(21) Application number: 10702252.7
(22) Date of filing: 28.01.2010
(51) Int. Cl.: C22C 47/14, C22C 49/14, C01B 31/02, C22C 49/06

(54) **A CONNECTION MEANS, A METHOD OF MANUFACTURING THE SAME AND A MATERIAL CONNECTION**
VERBINDUNGSMITTEL, HERSTELLUNGSVERFAHREN DAFÜR UND MATERIALVERBINDUNG
MOYEN DE CONNEXION, PROCÉDÉ DE FABRICATION ASSOCIÉ ET CONNEXION DE MATÉRIAU

(30) Priority: 16.02.2009 DE 102009009110; 17.09.2009 WO PCT/EP2009/006737
(43) Date of publication of application: 21.12.2011
(73) Proprietor: Bayer International SA, 1701 Fribourg (CH)
(72) Inventor: ZOZ, Henning, 57482 Wenden (DE); DVORAK, Michael, 3608 Thun (CH); ADAMS, Horst, 9450 Altstätten (CH)
(74) Representative: Klimiuk, Meike
(86) International application number: PCT/EP2010/000521
(87) International publication number: WO 2010/091791

(56) References cited:
- EP-A1- 1 918 249
- WO-A1-2009/010297
- WO-A2-2005/065281
- EDTMAIER C ET AL: "ALUMINIUM BASED CARBON NANOTUBE COMPOSITES BY MECHANICAL ALLOYING" PM POWDER METALLURGY WORLD CONGRESS PROCEEDINGS, XX, XX, 17 October 2004 (2004-10-17), pages 1-6, XP001248891 cited in the application
- GEORGE ET AL: "Strengthening in carbon nanotube/aluminium (CNT/Al) composites" SCRIPTA MATERIALIA, ELSEVIER, AMSTERDAM, NL, vol. 53, no. 10, 1 November 2005 (2005-11-01), pages 1159-1163, XP005045925 ISSN: 1359-6462 cited in the application
- ESAWI A ET AL: "Dispersion of carbon nanotubes (CNTs) in aluminum powder" COMPOSITES, IPC BUSINESS PRESS LTD. HAYWARDS HEATH, GB, vol. 38, no. 2, 23 June 2006 (2006-06-23), pages 646-650, XP002413866 ISSN: 0010-4361 cited in the application

## Description

### TECHNICAL FIELD

The present invention relates to a connection means made from metal, and in particular a light metal such as Al, Mg, Cu, Ti or an alloy comprising one or more of the same. The invention also relates to a method for producing the same and a material connection employing the connection means.

### BACKGROUND ART

There is a continuous demand in the art for connection means such as screws, bolts, hinges or rivets. In many applications, the ideal connection means would have a small weight, a high strength such as a high Vickers hardness and a high tensile strength, a high temperature stability and a high corrosion resistance.

Unfortunately, currently none of the known connection means provides for all of the above advantageous characteristics, instead prior art connection means will always resemble some sort of compromise in this regard. For example, in some cases Al-based alloys due to their low weight are used for manufacturing connection means. Unfortunately, many high strength Al-alloys have an inferior corrosion resistivity and they can often not be anodized. Also, many high strength aluminum alloys need a heat treatment to obtain the desired mechanical properties, which often will only be permanent in relatively small temperature ranges. This is especially crucial since the deterioration in the mechanical properties after use at higher temperatures is non-reversible.

The reduced temperature stability of such high strength aluminum alloys also implies that they can often only be processed by cold working or machining. Unfortunately, in cold working, tensions build up inside the metal matrix which have to be reduced by thermal processing. What is more, in the course of the thermal processing, dimensional consistency of high precision pieces cannot be guaranteed. On the other hand, manufacturing connection means such as screws by machining is not only very costly, but also leads to unfavourable geometrical tension distributions which often lead to a decreased strength with regard to shear forces.

Accordingly, most of the highest strength aluminum alloys are not suitable for connection means, are costly in production and still have to be protected against corrosion.

On the other hand, a number of corrosion resistant Al-alloys are known which are based on solid-solution strengthening, such as the series Al1xxx, Al3xxx and Al5xxx according to standard EN 573-3/4, which usually can also be anodized. However, the mechanical strengths of these alloys are rather poor and can only be increased in narrow limits by work hardening.

It is thus an object of the invention to provide a connection means which is light-weight, corrosion resistant and has a high mechanical strength, in particular a high Vickers hardness and a high tensile strength.

It is also an object of the invention to provide for a method of manufacturing said connection means which is suitable for mass production at rather moderate costs.

### SUMMARY OF THE INVENTION

In order to meet the above objects, a connection means made from metal, and in particular a light metal such as Al, Mg, Cu Ti or an alloy comprising one or more of the same is provided, which is made from a compound material of said metal reinforced by nanoparticles, in particular CNT, wherein the reinforced metal has a microstructure comprising metal crystallites at least partly separated by nanoparticles. Herein, the compound preferably comprises metal crystallites having a size in a range of 1 nm to 100 nm, preferably 10 nm to 100 nm, or in a range of more than 100 nm and up to 200 nm.

In the following, specific reference will be made to CNT as said nanoparticles for simplicity. It is however believed that similar effects could also be achieved when using other types of nanoparticles having a high aspect ratio, in particular inorganic nanoparticles such as carbides, nitrides and silicides. Thus, wherever applicable every disclosure made herein with respect to CNT is also contemplated with reference to other types of nanoparticles having a high aspect ratio, without further mention.

The structure of the material constituting the connection means has a new and surprising effect in that the micro structure of the metal crystallites is stabilized by the nanoparticles (CNT). In particular, it has been observed that due to a positioning of the CNT along the grain boundaries of the small, preferably nano scale metal crystallites, a dislocation movement can be suppressed and dislocations in the metal can be stabilized by the CNT. This stabilization is very effective due to the extremely high surface to volume ratio of the nano scale crystallites. Also, if alloys strengthened by solid-solution hardening are used as the metal constituents, the phases of the mixed crystal or solid solution can be stabilized by the engagement or interlocking with the CNT. Accordingly, this new effect which is observed to arise for small metal crystallites in combination with uniformly and preferably isotropically dispersed CNT is called "nano-stabilization" or "nano-fixation" herein. A further aspect of the nano-stabilization is that the CNT suppress a grain growth of the metal crystallites.

While the nano-stabilization is of course a microscopical (or rather nanoscopical) effect, it allows to produce a compound material as an intermediate product and to further manufacture a finished connection means therefrom having unprecedented macroscopic mechanical properties. First of all, the compound material will have a mechanical strength that is significantly higher than that of the pure metal component. A further surprising technical effect is an increased high-temperature stability of the compound material as well as of the connection means produced therefrom. For example, it has been observed that due to the nano-stabilization of the nano crystallites by CNT, a dislocation density and an increased hardness associated therewith can be conserved at temperatures close to the melting point of some of the phases of the metal. This means that the connection means can be produced by hot working or extrusion methods at temperatures close to the melting point of some of the phases of the metal while preserving the mechanical strength and hardness of the compound. For example, if the metal is aluminum or an aluminum alloy, the person skilled in the art will appreciate that hot working would be an untypical way of processing it, since this would usually severely compromise the mechanical properties of the aluminum. However, due to the nano-stabilization described above, an increased Young modulus and hardness will be preserved even under hot working. By the same token, the final connection means formed from the nano-stabilized compound as a source material can be used for high-temperature applications, such as engines or turbines, where light metals typically fail due to lack of high-temperature stability.

In some embodiments of the invention, the nanoparticles are not only partly separated from each other by the CNT, but some CNT are also contained or embedded in crystallites. One can think of this as a CNT sticking out like a "hair" from a crystallite. These embedded CNTs are believed to play an important role in preventing grain growth and internal relaxation, i.e. preventing a decrease of the dislocation density when energy is supplied in form of pressure and/or heat upon compacting the compound material. Using mechanical alloying techniques of the type as described below, it is possible to produce crystallites below 100 nm in size with embedded CNTs. In some instances, depending on the diameter of the CNTs, it may be easier to embed the CNTs in crystallites ranging between 100 nm and 200 nm in size. In particular, with the additional stabilization effect for the embedded CNTs, the nano-stabilisation has been found to be very effective also for crystallites between 100 nm and 200 nm in size.

As regards aluminum as a metal component of the connection means, the invention allows to circumvent many problems currently encountered with Al alloys. While high strength Al alloys are known, such as Al7xxx incorporating Zinc or Al8xxx incorporating Li according to Standard EN 573-3/4, unfortunately, coating these alloys by anodic oxidation proves to be difficult. Also, if different Al alloys are combined, due to a different electro-chemical potentials of the alloys involved, corrosion may occur in the contact region. On the other hand, while Al alloys of the series 1xxx, 3xxx and 5xxx based on solid-solution hardening can be coated by anodic oxidation, they have comparatively poor mechanical properties, a low temperature stability and can only be hardened to a quite narrow degree by cold working.

In contrast to this, if pure aluminum or an aluminum alloy is used as the metal constituent of the composite material of the connection means, an aluminum based composite material can be provided which due to the nano-stabilization effect has a strength and hardness comparable with or even beyond the highest strength aluminum alloy available today, which also has an increased high-temperature strength due to the nano-stabilization and is open for anodic oxidation. If a high-strength aluminum alloy is used as the metal of the composite of the invention, the strength of the compound can even be further raised. Also, by adequately adjusting the percentage of CNT in the composite, the mechanical properties can be adjusted to a desired value. Therefore, materials having the same metal component but different concentrations of CNT and thus different mechanical properties can be manufactured, which will have the same electro-chemical potential and therefore will not be prone to corrosion when connected with each other. This is different from prior art, where different alloys need to be used when different mechanical properties are needed, and where accordingly corrosion is always an issue when different alloys are brought in contact.

The present invention also provides a material connection comprising a first part, a second part and a connection means connecting the first and second parts, wherein at least one of said first and second parts comprises a metal or a metal alloy. In many situations, it will be necessary that the connection means has different, in particular superior mechanical properties as compared with the first and second parts that are to be connected thereby. Traditionally, this would imply that the connection means would be a metal or a metal alloy different from the metal or metal alloy of the first and/or second part having the desired mechanical properties in order to compensate for instance for different thermal expansion coefficients for the two parts to be connected. However, since the chemical potentials between the first and second part and of the connection means will generally be different, the connection means will act as a galvanic element with regard to the parts, thus leading to contact corrosion in presence of an electrolyte.

In contrast, since the mechanical properties of the connection means of the invention can be adjusted by the content of nanoparticles, it is in many cases possible to use the same metal component in the connection means as in the parts to be connected thereby and to still obtain suitable different mechanical properties. This way, contact corrosion between the first and second part on the one hand and the connection means on the other hand can be reliably avoided.

As a matter of fact, it is not necessary that the metal component of the first and/or second parts and the connection means are identical, but in practice it will be sufficient that the respective chemical potentials deviate by less than 50 mV, preferably less than 25 mV from each other.

In summary, since in the connection means of the invention, the content of nanoparticles can be controlled to adjust the desired mechanical properties rather than the metal content used, this additional degree of freedom can be advantageously used to provide material connections employing a connection means which is both compatible with the parts to be connected from an electrochemical point of view and still provides the desired mechanical properties, which due to the nanoparticle content can be very different from that of the parts to be connected.

It has indeed been found that the tensile strength and the hardness can be varied approximately proportionally in a wide range with the content of CNT in the composite material. For light metals, such as aluminum, it has been found that the Vickers hardness increases nearly linearly with the CNT content. At a CNT content of above about 10.0wt%, the composite material becomes extremely hard and brittle. Accordingly, depending on the desired mechanical properties, a CNT content from 0.5 to 10.0wt% will be preferable. In particular, a CNT content in the range of 2.0 to 9.0% is extremely useful as it allows to make composite materials of extraordinary strength in combination with the aforementioned advantages of nano-stabilization, in particular high-temperature stability.

As has been explained above, according to one aspect of the invention, the mechanical properties of the connection means connecting a first and a second part can be specifically adapted without the necessity to use a different metal component, but by varying the nanoparticle content instead. The same principle is of course also applicable with regard to the first and second parts themselves, which each may be made from a compound material comprising metal or a metal alloy and nanoparticles, and where the mechanical properties of the two parts may be different due to different contents of nanoparticles. In a preferred embodiment, the numerical value of nanoparticles by weight of the first and second parts differ at least by 10%, preferably by at least 20% of the higher one of said numerical values. Thus, if the percentage of nanoparticles by weight would be 5% for the first part and 4% for the second part, the numerical values of the percentages would differ by 20% of the higher one of said numerical values.

This concept may be pushed even one step further by providing an integral part made from a compound material of a metal or metal alloy reinforced be nanoparticles, wherein the concentration of nanoparticles varies between different regions of the integral part. For example, if the part would be a plate, the nanoparticle content could monotonously increase along a length or width direction between a first and a second end of the plate, which would mean that the plate would have an increased tensile strength or Vickers hardness in a region close to its second end as compared to a region close to its first end.

Note that the same materials, the same mechanical properties and the same manufacturing methods described herein with connection to connection means equally apply with regard to the integral part, without further mention. In particular, the same type of composite powder material that will be described below and the same type of compacting methods thereof may equally be applied with regard to the integral part, while the explicit description thereof is omitted for brevity.

It is mentioned that compound metal/CNT materials per se are for example from US 2007/0134496 A1, JP 2007/154 246 A, WO 2006/123 859 A1, WO 2008/052 642, WO 2009/010 297 and JP 2009/030 090. A detailed discussion thereof is made in the priority application PCT/EP2009/006 737, which is included herein by reference.

Also, in the priority application PCT/EP2009/006 737 an overview over prior art with regard to production of CNT is given, which is likewise included herein by reference

When the connection means based on CNT reinforced metal are to be manufactured, there is a problem arising in prior art which is related to possible exposure when handling CNTs (see e.g. Baron P. A. (2003) "Evaluation of Aerosol Release During the Handling of Unrefined Single Walled Carbon Nanotube Material", NIOSH DART-02-191 Rev. 1.1 April 2003; Maynard A. D. et al. (2004) "Exposure To Carbon Nanotube Material: Aerosol Release During The Handling Of Unrefined Singlewalled Carbon Nanotube Material", Journal of Toxicology and Environmental Health, Part A, 67:87-107; Han, J. H. et al. (2008) 'Monitoring Multiwalled Carbon Nanotube Exposure in Carbon Nanotube Research Facility', Inhalation Toxicology, 20:8, 741 - 749).

According to a preferred embodiment, this can be minimized by providing the CNT in form of a powder of tangled CNT-agglomerates having a mean size sufficiently large to ensure easy handling because of a low potential dustiness. Herein, preferably at least 95% of the CNT-agglomerates have a particle size larger than 100 µm. Preferably, the mean diameter of the CNT-agglomerates is between 0.05 and 5 mm, preferably 0.1 and 2 mm and most preferably 0.2 and 1 mm.

Accordingly, the nanoparticles to be processed with the metal powder can be easily handled with the potential for exposure being minimized. With the agglomerates being larger than 100 µm, they can be easily filtered by standard filters, and a low respirable dustiness in the sense of EN 15051-B can be expected. Further, the powder comprised of agglomerates of this large size has a pourability and flowability which allows an easy handling of the CNT source material.

While one might expect at first sight that it could be difficult to uniformly disperse the CNT on a nano scale while providing them in the form of highly entangled agglomerates on a millimetre scale, it has been confirmed by the inventors that a homogeneous and isotopic dispersion throughout the compound is in fact possible using mechanical alloying, which is a process of repeated deformation, fraction and welding of the metal and CNT particles. In fact, as will be explained below with reference to a preferred embodiment, the tangled structure and the use of large CNT-agglomerates even helps to preserve the integrity of the CNT upon the mechanical alloying at high kinetic energies.

Further, the length-to-diameter ratio of the CNT, also called aspect ratio, is preferably larger than 3, more preferably larger than 10 and most preferably larger than 30. A high aspect ratio of the CNT again assists in the nano-stabilization of the metal crystallites.

In an advantageous embodiment of the present invention, at least a fraction of the CNTs have a scrolled structure comprised of one or more rolled up graphite layers, each graphite layer consisting of two or more graphene layers on top of each other. This type of nano tubes has for the first time been described in DE 10 2007 044 031 A1 which has been published after the priority date of the present application. This new type of CNT structure is called a "multi-scroll" structure to distinguish it from "single-scroll" structures comprised of a single rolled-up graphene layer. The relationship between multi-scroll and single-scroll CNTs is therefore analogous to the relationship between single-wall and multi-wall cylindrical CNTs. The multi-scroll CNTs have a spiral shaped cross section and typically comprise 2 or 3 graphite layers with 6 to 12 graphene layers each.

The multi-scroll type CNTs have found to be extraordinarily suitable for the above mentioned nano-stabilization. One of the reasons is that the multi-scroll CNT have the tendency to not extend along a straight line but to have a curvy or kinky, multiply bent shape, which is also the reason why they tend to form large agglomerates of highly tangled CNTs. This tendency to form a curvy, bent and tangled structure facilitates the formation of a three-dimensional network interlocking with the crystallites and stabilizing them.

A further reason why the multi-scroll structure is so well suited for nano-stabilization is believed to be that the individual layers tend to fan out when the tube is bent like the pages of an open book, thus forming a rough structure for interlocking with the crystallites which in turn is believed to be one of the mechanisms for stabilization of defects.

Further, since the individual graphene and graphite layers of the multi-scroll CNT apparently are of continuous topology from the center of the CNT towards the circumference without any gaps, this again allows for a better and faster intercalation of further materials in the tube structure, since more open edges are available forming an entrance for intercalates as compared to single-scroll CNTs as described in Carbon 34, 1996, 1301 - 03, or as compared to CNTs having an onion type structure as described in Science 263, 1994, 1744 - 47.

In a preferred embodiment, at least a fraction of the nanoparticles are functionalized, in particular roughened prior to the mechanical alloying. When the nanoparticles are formed by multi-wall or multi-scroll CNTs, the roughening may be performed by causing at least the outermost layer of at least some of the CNTs to break by submitting the CNTs to high pressure, such as a pressure of 5.0 MPa or higher, preferably 7.8 MPa or higher, as will be explained below with reference to a specific embodiment. Due to the roughening of the nanoparticles, the interlocking effect with the metal crystallites and thus the nano-stabilization is further increased.

In a preferred embodiment, the processing of the metal particles and the nanoparticles is conducted such as to increase and stabilize the dislocation density of the crystallites by the nanoparticles sufficiently to increase the average Vickers hardness of the composite material to exceed the Vickers hardness of the original metal by 40% or more, preferably by 80% or more.

Also, the processing is conducted such as to stabilize the dislocations, i.e. suppress dislocation movement and to suppress the grain growth sufficiently such that the Vickers hardness of the connection means formed by compacting the composite powder is higher than the Vickers hardness of the original metal, and preferably higher than 80% of the Vickers hardness of the composite powder.

The high dislocation density is preferably generated by causing numerous high kinetic energy impacts of balls of a ball mill. Preferably, in the ball mill the balls are accelerated to a speed of at least 8.0 m/s, preferably at least 11.0 m/s. The balls may interact with the processed material by shear forces, friction and collision forces, but the relative contribution of collisions to the total mechanical energy transferred to the material by plastic deformation increases with increasing kinetic energy of the balls. Accordingly, a high velocity of the balls is preferred for causing a high rate of kinetic energy impacts which in turn causes a high dislocation density in the crystallites.

Preferably, the milling chamber of ball mill is stationary and the balls are accelerated by a rotary motion of a rotating element. This design allows to easily and efficiently accelerate the balls to the above mentioned velocities of 8.0 m/s, 11.0 m/s or even higher, by driving the rotating element at a sufficient rotary frequency such that the tips thereof are moved at the above mentioned velocities. This is different from, for example, ordinary ball mills having a rotating drum or planetary ball mills, where the maximum speed of the balls is typically 5 m/s only. Also, the design employing a stationary milling chamber and a driven rotating element is easily scaleable, meaning that the same design can be used for ball mills of very different sizes, from laboratory type mill up to mills for high throughput mechanical alloying on an industrial scale.

Preferably, the axis of the rotary element is oriented horizontally, such that the influence of gravity on both, the balls and the processed material, is reduced to a minimum.

In a preferred embodiment, the balls have a small diameter of 3.0 to 8.0 mm, preferably 4.0 to 6.0 mm. At this small ball diameters, the contact zones between the balls are nearly point shaped thus leading to very high deformation pressures, which in turn facilitates the formation of a high dislocation density in the metal.

The preferred material of the balls is steel, ZiO₂ or yttria stabilized ZiO₂.

The quality of the mechanical alloying will also depend on the filling degree of the milling chamber with the balls as well as on the ratio of balls and processed material. Good mechanical alloying results can be achieved if the volume occupied by the balls roughly corresponds to the volume of the chamber not reached by the rotating element. Thus, the filing degree of the balls is preferably chosen such that the volume *V_{b}* occupied by the balls corresponds to *V_{b}* = *V_{c}* - π · (r*_{R}*)² · *l* ± 20% , wherein *V_{c}* is the volume of the milling chamber, *r_{R}* is the radius of the rotating element and I is the length of the milling chamber in axial direction of the rotor. Also, the ratio of the processed material, i.e. (metal + nanoparticles) / balls by weight is preferably between 1:7 and 1:13.

While milling with high kinetic energy is advantageous with regard to increasing the dislocation density in the metal crystallites, high kinetic energies in practice lead to two severe problems. The first problem is that many metals due to their ductility will tend to stick to the balls, the chamber walls or the rotating element and thus not be processed further. This is especially true for light metals such as Al. Consequently, the part of the material that is not completely processed will not have the desired quality of the nano-stabilized CNT-metal composite, and the quality of products formed therefrom may be locally deficient, which may lead to breakage or failure of the finished article. Accordingly, it is of high importance that all of the material is completely and uniformly processed.

The second problem encountered when processing at high kinetic energies is that the CNT may be worn down or destroyed to an extent that the interlocking effect with the metal crystallites, i.e. the nano-stabilization no longer occurs.

To overcome these problems, in a preferred embodiment of the invention, the processing of the metal and the CNTs comprises a first and a second stage, wherein in the first processing stage most or all of the metal is processed and in the second stage CNTs are added and the metal and the CNTs are simultaneously processed. Accordingly, in the first stage, the metal can be milled down at high kinetic energy to a crystallite size of 100 nm or below before the CNTs are added, such as to not wear down the CNT in this milling stage. Accordingly, the first stage is conducted for a time suitable to generate metal crystallites having an average size in a range of 1 to 100 nm, which in one embodiment was found to be a time of 20 to 60 minutes. The second stage is then conducted for a time sufficient to cause a stabilization of the nanostructure of the crystallites, which may typically take 5 to 30 min only. This short time of the second stage is sufficient to perform mechanical alloying of the CNT and the metal and to thereby homogeneously disperse the CNT throughout the metal matrix, while not yet destroying too much of the CNT.

In order to avoid sticking of the metal during the first stage, it has proven to be very efficient to add some CNTs already during the first stage which may then serve as a milling agent preventing sticking of the metal component. This fraction of the CNT will be sacrificed, as it will be completely milled down and will not have any noticeable nano-stabilizing effect. Accordingly, the fraction of CNT added in the first stage will be kept as small as possible as long as it prevents sticking of the metal constituent.

In a further preferred embodiment, during the processing, the rotation speed of the rotating element is cyclically raised and lowered. This technique is for example described in DE 196 35 500 and referred to as "cycle operation". It has been found that by conducting the processing with alternating cycles of higher and lower rotational speeds of the rotating element, sticking of the material during processing can be very efficiently be prevented. The cycle operation, which is per se known for example from the above referenced patent has proven to be very useful for the specific application of mechanical alloying of a metal and CNTs.

The method of manufacturing the connection means may also comprise the manufacturing of CNTs in the form of CNT powder as a source material. The method may comprise a step of producing the CNT powder by catalytic carbon vapor deposition using one or more of a group consisting of acetylene, methane, ethane, ethylene, butane, butene, butadylene, and benzene as a carbon donor. Preferably, the catalyst comprises two or more elements of a group consisting of Fe, Co, Mn, Mo and Ni. It has been found that with these catalysts, CNTs can be formed at high yield, allowing a production on an industrial scale. Preferably, the step of producing the CNT powder comprises a step of catalytic decomposition of C₁-C₃-carbo hydrogens at 500°C to 1000°C using a catalyst comprising Mn and Co in a molaric ratio in a range of 2:3 to 3:2. With this choice of catalyst, temperature and carbon donor, CNTs can be produced at high yield and in particular, in the shape of large agglomerates and with the preferred multi-scroll morphology.

### BRIEF DESCRIPTION OF THE FIGURES

- Fig. 1: is a schematic diagram illustrating the production setup for high quality CNTs.
- Fig.2: is a sketch schematically showing the generation of CNT-agglomerates from agglomerated primary catalyst particles.
- Fig. 3: is an SEM picture of a CNT-agglomerate.
- Fig. 4: is a close-up view of the CNT-agglomerate of Fig. 3 showing highly entangled CNTs.
- Fig. 5: is a graph showing the size distribution of CNT-agglomerates obtained with a production setup shown in Fig. 1
- Fig. 6a: is an SEM image of CNT-agglomerates prior to functionalization.
- Fig. 6b: is an SEM image of the same CNT-agglomerates after functionalization.
- Fig. 6c: is a TEM image showing a single CNT after functionalization.
- Fig. 7: is a schematic diagram showing a setup for spray atomization of liquid alloys into an inert atmosphere.
- Figs. 8a and 8b: show sectional side and end views respectively of a ball mill designed for high energy milling.
- Fig. 9: is a conceptional diagram showing the mechanism of mechanical alloying by high energy milling.
- Fig. 10: is a diagram showing the rotational frequency of the HEM rotor versus time in a cyclic operation mode.
- Fig. 11a: shows the nano structure of a compound of the invention in a section through a compound particle.
- Fig. 11b: shows, in comparison to Fig. 11a, a similar sectional view for the compound material as known from WO 2008/052642 A1 and WO 2009/010297 A1.
- Fig. 12: shows an SEM image of the composite material according to an embodiment of the invention in which CNTs are embedded in metal crystallites.
- Fig. 13: shows a schematic diagram of a material connection employing a connection means according to an embodiment of the invention
- Fig. 14: shows a schematic diagram of a material connection between four parts made from compound materials of metal reinforced by different concentrations of nanoparticles connected by connection means according to an embodiment of the present invention.
- Fig. 15: shows a schematic diagram of an integral part made from metal reinforced by nanoparticles, wherein the concentration of nanoparticles varies between different regions of the integral part.

### DESCRIPTION OF A PREFERRED EMBODIMENT

For the purposes of promoting an understanding of the principles of the invention, reference will now be made to the preferred embodiment illustrated in the drawings and specific language will be used to describe the same. It will, nevertheless, be understood that no limitation of the scope of the invention is thereby intended, such alterations and further modifications in the illustrated connection means, method and use and such further applications of the principles of the invention as illustrated therein being contemplated as would normally occur now or in the future to one skilled in the art to which the invention relates.

In the following, a processing strategy for manufacturing connection means according to an embodiment of the invention is summarized. For this, a method of producing constituent materials and of producing a composite material from the constituent materials will be explained. Also, different ways of compacting the composite material such as to form a connection means or a blank for a connection means will be discussed.

In the preferred embodiment, the processing strategy comprises the following steps:
1.) production of high quality CNTs,
2.) functionalization of the CNTs,
3.) spray atomisation of liquid metal or alloys into inert atmosphere,
4.) high energy milling of metal powders,
5.) mechanical dispersion of CNTs in the metal by mechanical alloying,
6.) compacting of metal-CNT composite powders to form connection means or blanks thereof, and
7.) further processing of compacted connection means or blanks.

Preferred embodiments of the above steps are described in detail below. Also, a material connection employing a connection means thus produced will be shown below.

### 1. PRODUCTION OF HIGH QUALITY CNTS

In Fig. 1, a setup 10 for producing high quality CNTs by catalytic CVD in a fluidized bed reactor 12 is shown. The reactor 12 is heated by heating means 14. The reactor 12 has a lower entrance 16 for introducing inert gases and reactant gases, an upper discharge opening 18 for discharging nitrogen, inert gas and by-products from the reactor 12, a catalyst entrance 20 for introducing a catalyst and a CNT discharge opening 22 for discharging CNTs formed in the reactor 12.

In a preferred embodiment, CNTs of the multi-scroll type are produced by a method as known from DE 10 2007 044 031 A1, which has been published after the priority date of the present application and the whole content of which is hereby included in the present application by reference.

First, nitrogen as an inert gas is introduced in the lower entrance 16 while the reactor 12 is heated by heating means 14 to a temperature of 650°C.

Next, a catalyst is introduced through catalyst entrance 20. Herein, the catalyst is preferably a transition metal catalyst based on Co and Mn, wherein the molaric ratio of Co and Mn with respect to each other is between 2:3 and 3:2.

Next, a reactant gas is introduced at the lower entrance 16, comprising a hydrocarbon gas as a carbon donor and an inert gas. Herein, the hydrocarbon gas preferably comprises C₁-C₃-carbo-hydrogens. The ratio of reactant and inert gas may be about 9:1.

Carbon deposited in form of CNT is discharged at the CNT discharge opening 22.

The catalyst material is typically milled to a size of 30 to 100 µm. As is shown in schematically in Fig. 2, a number of primary catalyst particles may agglomerate and carbon is deposited by CVD on the catalyst particle surfaces such that CNTs are grown. According to the preferred production method of the invention, the CNT form agglomerates of long entangled fibres upon growth, as is schematically shown in the right half of Fig. 2. At least part of the catalyst will remain in the CNT-agglomerate. However, due to the very rapid and efficient growth of the CNT, the catalyst content in the agglomerates will become negligible, as the carbon content of the agglomerates may eventually be higher than 95%, in some embodiments even higher than 99%.

In Fig. 3, an SEM image of a CNT-agglomerate thus formed is shown. The agglomerate is very large by "nano-standards", having a diameter of more than 1 mm. Fig. 4 shows an enlarged image of the CNT-agglomerate, in which a multitude of highly entangled CNTs with a large length to diameter ratio can be seen. As can be seen from Fig. 4, the CNTs have a "curly" or "kinky" shape, as each CNT has only comparatively short straight sections with numerous bends and curves inbetween. It is believed that this curliness or kinkiness is related to the peculiar structure of the CNTs, which is called the "multi-scroll structure" herein. The multi-scroll structure is a structure comprised of one or more rolled up graphite layers, where each graphite layer consists of two or more graphene layers on top of each other. This structure has for the first time been reported in DE 10 2007 044 031 A1 published after the priority date of the present application.

The below Table 1 summarizes the characteristic properties of high purity multi-scroll CNT that have been produced with the setup of Fig. 1.

**Table 1**

| **Properties** | **Value** | **Unit** | **Method** |
|---|---|---|---|
| **C-Purity** | >95 | wt% | ashing |
| **Free amorphous carbon** | - | wt% | TEM |
| **Outer mean diameter** | ~13 | nm | TEM |
| **Inner mean diameter** | ~4 | nm | TEM |
| **Length** | 1 ->10 | µm | SEM |
| **Bulk density** | 130 - 150 | kg/m³ | EN ISO 60 |

It is noted that the CNTs have a considerably high C-purity of more than 95wt%. Also, the average outer diameter is only 13 nm at a length of 1 to 10 µm, i.e. the CNTs have a very high aspect ratio. A further remarkable property is the high bulk density being in a range of 130 to 150 kg/m³. This high bulk density greatly facilitates the handling of the CNT-agglomerate powder, and allows easy pouring and efficient storing thereof. This is of great importance when it comes to application of the composite material for manufacturing connection means on an industrial scale.

The CNT-agglomerates with the properties of Table 1 can be produced rapidly and efficiently with a high throughput. Even today the applicant already has the capacity to produce 60 tons of this type of CNT-agglomerates per year.

Table 2 summarizes the same properties for a very high purity CNT-agglomerate which the applicant is also able to produce, although at a lower capacity.

**Table 2**

| **Properties** | **Value** | **Unit** | **Method** |
|---|---|---|---|
| **C-Purity** | >99 | wt% | ashing |
| **Free amorphous carbon** | - | wt% | TEM |
| **Outer mean diameter** | ~13 | nm | TEM |
| **Inner mean diameter** | ~4 | nm | TEM |
| **Length** | 1 ->10 | µm | SEM |
| **Bulk density** | 140 - 230 | kg/m³ | EN ISO 60 |

Fig. 5 shows a graph of the particle-size distribution of the CNT-agglomerates. The abscissa represents the particle size in µm, while the ordinate represents the cumulative volumetric content. As can be seen from the diagram in Fig. 5, almost all of the CNT-agglomerates have a size larger than 100 µm. This means that practically all of the CNT-agglomerates can be filtered by standard filters. These CNT-agglomerates have a low respirable dustiness under EN 15051-B. Thus, the extraordinarily large CNT-agglomerates used in the preferred embodiment of the invention allow for a safe and easy handling of the CNT, which again is of highest importance when it comes to transferring the technology from the laboratory to the industrial scale. Also, due to the large CNT-agglomerate size, the CNT powder has a good pourability, which also greatly facilitates the handling. Thus, the CNT-agglomerates allow to combine macroscopic handling properties with nanoscopic material characteristics.

### 2. FUNCTIONALIZATION OF CNT

In a preferred embodiment, the CNTs are functionalized prior to performing the mechanical alloying. The purpose of the functionalizing is to treat the CNTs such that the nano-stabilization of the metal crystallites in the composite material will be enhanced. In the preferred embodiment, this functionalization is achieved by roughening the surface of at least some of the CNTs.

Herein, the CNT-agglomerates as shown in Fig. 6a are submitted to a high pressure of 100 kg/cm² (9.8 MPa). Upon exerting this pressure, as is shown in Fig. 6b, the agglomerate structure as such is preserved, i.e. the functionalized CNTs are still present in the form of agglomerates preserving the aforementioned advantages with respect to low respirable dustiness and easier handling. Also, it is found that while the CNT retain the same inner structure, the outermost layer or layers burst or break, thereby developing a rough surface, as is shown in Fig. 6c. With the rough surface, the interlocking effect between CNT and crystallites is increased, which in turn increases the nano-stabilization effect.

### 3. METAL POWDER GENERATION THROUGH ATOMIZATION

In Fig. 7, a setup 24 for generating a metal powder through atomization is shown. The setup 24 comprises a vessel with heating means in which a metal or metal alloy to be used as a constituent of the composite material is melted. The liquid metal or alloy is poured into a chamber 30 and forced by argon driving gas, represented by an arrow 32 through a nozzle assembly 34 into a chamber 36 containing an inert gas. In the chamber 36, the liquid metal spray leaving the nozzle assembly 34 is quenched by an argon quenching gas 38, so that the metal droplets are rapidly solidified and form a metal powder 40 piling up on the floor of chamber 36. This powder forms the metal constituent of the composite material used for manufacturing connection means according to an embodiment of the invention.

### 4. HIGH ENERGY MILLING OF METAL POWDERS AND MECHANICAL DISPERSION OF CNT IN METAL

In order to form the composite material from the CNT produced as described in section 1 and functionalized as described in section 2 and from the metal powder produced as described in section 3, the CNTs need to be dispersed within the metal. In the preferred embodiment, this is achieved by a mechanical alloying carried out in a high energy mill 42, which is shown in a sectional side view in Fig. 8a and a sectional end view in Fig. 8b. The high energy mill 42 comprises a milling chamber 44 in which a rotating element 46 having a number of rotating arms 48 is arranged such that the rotary axis extends horizontally. While this is not shown in the schematic view of Fig. 8, the rotating element 46 is connected to a driving means such as to be driven at a rotational frequency of up to 1,500 RPM or even higher. In particular, the rotating element 46 can be driven at a rotational speed so that the radially outward lying tips of each arm 48 acquire a velocity of at least 8.0 m/s, preferably more than 11.0 m/s with respect to the milling chamber 44, which itself remains stationary. Although not shown in Fig. 8, a multitude of balls are provided in the milling chamber 44 as milling members. A close-up look of two balls 50 is shown in Fig. 9 to be described in more detail below. In the present example, the balls are made from steel and have a diameter of 5.1 mm. Alternatively, the balls 50 could be made from ZiO₂ or yttria stabilized said ZiO₂.

The filling degree of the balls within the high energy mill 42 is chosen such that the volume occupied by the balls corresponds to the volume of the milling chamber 44 that lies outside the cylindrical volume that can be reached by the rotating arms 48. In other words, the volume *V_{b}* occupied by the balls corresponds to *V_{b}* = *V_{c}* - π *·* (r*_{R}*)² · *l*, wherein *V_{c}* is the volume of the milling chamber 44, *r_{R}* is the radius of the rotating arms 48 and *r* is the length of the milling chamber 44 in axial direction. Similar high energy ball mills are disclosed in DE 196 35 500, DE 43 07 083 and DE 195 04 540 A1.

The principle of mechanical alloying is explained with reference to Fig. 9. Mechanical alloying is a process where powder particles 52 are treated by repeated deformation, fracture and welding by highly energetic collisions of grinding balls 50. In the course of the mechanical alloying, the CNT-agglomerates are deconstructed and the metal powder particles are fragmentized, and by this process, single CNTs are dispersed in the metal matrix. Since the kinetic energy of the balls depends quadratically on the velocity, it is a primary object to accelerate the balls to very high velocities of 10 m/s or even above. The inventors have analyzed the kinetics of the balls using high speed stroboscopic cinematopography and could confirm that the maximum relative velocity of the balls corresponds approximately to the maximum velocity of the tips of the rotating arms 48.

While in all types of ball mills the processed media are subjected to collision forces, shear forces and frictional forces, at higher kinetic energies the relative amount of energy transferred by collision increases. In the framework of the present invention, it is preferred that from the total mechanical work applied to the processed media, the relative contribution of collisions is as high as possible. For this reason, the high energy ball mill 42 shown in Fig. 8 is advantageous over ordinary drum-ball mills, planetary ball mills or attritors since the kinetic energy of the balls that can be reached is higher. For example, in a planetary ball mill or in an attritor, the maximum relative velocity of the balls is typically 5 m/s or below. In a drum-ball mill, where the balls are set in motion by rotation of the milling chamber, the maximum velocity of the balls will depend both on the rotational velocity and the size of the milling chamber. At low rotational speeds, the balls are moved in the so called "cascade mode", in which the frictional and shear forces dominate. At higher rotational frequencies, the ball motion enters the so called "cataract mode", in which the balls are accelerated due to gravity in a free fall mode, and accordingly, the maximum velocity will depend on the diameter of the ball mill. However, even for the largest drum-ball mills available, the maximum velocity will hardly surpass 7 m/s. Accordingly, the HEM design with a stationary milling chamber 44 and a driven rotating element 46 as shown in Fig. 8 is preferred.

When processing the metal powder at high kinetic energies, this has two effects that are connected with the strengthening of the composite material. The first effect is a decrease of crystallite size. According to the Hall-Petch equation, the yield stress σ*_{y}* increases inversely proportional with the square root of the crystallite diameter d, i.e. ${σ}_{y} = {σ}_{o} + \frac{{K}_{y}}{\sqrt{d}} ,$ wherein *K_{y}* is a material constant and σ₀ is the yield stress of the perfect crystal, or in other words, the resistance of the perfect crystal to dislocation motion. Accordingly, by decreasing the crystallite size, the material strength can be increased.

The second effect on the metal due to high energy collision is a work hardening effect due to an increase of dislocation density in the crystallites. The dislocations accumulate, interact with each other and serve as pinning points or obstacles that significantly impede their motion. This again leads to an increase in the yield strength σ*_{y}* of the material and a subsequent decrease in ductility.

Mathematically, the correlation between yield strength σ*_{y}* and dislocation density ρ can be expressed as follows: ${σ}_{y} = G ⋅ α ⋅ b ⋅ \sqrt{ρ} ,$ where G is the shear modulus, b is the Burger's vector and a is a material specific constant.

However, many metals, in particular light metals such as aluminum have a fairly high ductility which makes processing by high energy milling difficult. Due to the high ductility, the metal may tend to stick at the inside wall of the milling chamber 44 or the rotating element 46 and may thereby not be completely milled. Such sticking can be counteracted by using milling aids such as stearin acids or the like. In WO 2009/010297 by the same inventors, it was explained that the CNT itself may act as a milling agent which avoids sticking of the metal powder. However, when the metal powder and the CNT are milled simultaneously at sufficient energy and for a sufficient duration such as to decrease the metal crystallite size to 100 nm or below, the CNT will tend to be damaged to a degree that the envisaged nano-stabilization is greatly compromised.

According to a preferred embodiment, the high energy milling is therefore conducted in two stages. In a first stage, the metal powder and only a fraction of the CNT powder are processed. This first stage is conducted for a time suitable to generate metal crystallites having an average size below 200 nm, preferably below 100 nm, typically for 20 to 60 min. In this first stage, a minimum amount of CNT is added that will allow to prevent sticking of the metal. This CNT is sacrificed as a milling agent, i.e. it will not have a significant nano-stabilizing effect in the final composite material.

In a second stage, the remaining CNT is added and the mechanical alloying of the CNTs and the metal is performed. In this stage, the microscopic agglomerates as shown in Fig. 3 and Fig. 6b need to be decomposed into single CNTs which are dispersed in the metal matrix by mechanical alloying. In experiments, it has been confirmed that it is in fact easily possible to deconstruct the CNT alloy by high energy milling, which would be difficult to achieve in alternative dispersion methods. Also, it has been observed that the integrity of the CNTs added during the second stage in the metal matrix is very good, thus allowing for the nano-stabilization effect. As regards the integrity of the disentangled CNTs in the metal matrix, it is believed that using agglomerates of larger size is even advantageous, since the CNTs inside the agglomerates are to a certain extent protected by the outside CNTs.

Further, in the first stage the rotational speed of the rotational element 46 is preferably cyclically raised and lowered as is shown in the timing diagram of Fig. 10. As is seen in Fig. 10, the rotating speed is controlled in alternating cycles, namely a high speed cycle at 1,500 rpm for the duration of 4 min and a low speed cycle at 800 rpm for a duration of one minute. This cyclic modulation of rotating speed is found to impede sticking. Such cycle operation has already been described in DE 196 35 500 and has been successfully applied in the framework of the present invention.

By the above described process, a powder composite material can be obtained in which metal crystallites having a high dislocation density and a mean size below 200 nm, preferably below 100 nm are at least partially separated and micro-stabilized by homogeneously distributed CNTs. Fig. 11 a shows a cut through a composite material particle according to an embodiment of the invention. In Fig. 11a, the metal constituent is aluminum and the CNTs are of the multi-scroll type obtained in a process as described in section 1 above. As can be seen from Fig. 11a, the composite material is characterized by an isotropic distribution of nanoscopic metal crystallites located in a CNT mesh structure. In contrast to this, the composite material of WO 2008/052642 shown in Fig. 11b has a non-isotropic layer structure, leading to non-isotropic mechanical properties.

Fig. 12 shows an SEM image of a composite material comprised of aluminum with CNT dispersed therein. At locations denoted with number ①, examples of CNT extending along a boundary of crystallites can be seen. The CNTs separate individual crystallites from each other and thereby effectively suppress grain growth of the crystallites and stabilize the dislocation density. At locations marked with reference signs ②, CNTs can be seen which are contained or embedded within a nanocrystallite and stick out from the nanocrystallite surface like a "hair". It is believed that these CNTs have been pressed into the metal crystallites like needles in the course of the high energy milling described above. It is believed that these CNTs embedded or contained within individual crystallites play an important role in the nano-stabilization effect, which in turn is responsible for the superior mechanical properties of the composite material and of compacted articles formed thereby.

In the preferred embodiment, the composite powder is subjected to a passivation treatment in a passivation vessel (not shown). In this passivation, the finished composite powder is discharged from the milling chamber 42, while still under vacuum or in an inert gas atmosphere and is discharged into the passivation vessel. In the passivation vessel, the composite material is slowly stirred, and oxygen is gradually added such as to slowly oxidize the composite powder. The slower this passivation is conducted, the lower is the total oxygen uptake of the composite powder.

Passivation of the powder again facilitates the handling of the powder as a source material for fabrication of manufactured or semi-finished articles on an industrial scale.

### 5. COMPACTING OF THE COMPOSITE MATERIAL POWDER

The composite material powder is then used as a source material for forming semi-finished or finished connection means by powder metallurgic methods. In particular, it has been found that the powder material of the invention can very advantageously be further processed by cold isostatic pressing (CIP) and hot isostatic pressing (HIP). Alternatively, the composite material can be further processed by hot working, powder milling or powder extrusion at high temperatures close to the melting temperature of some of the metal phases. It has been observed that due to the nano-stabilizing effect of the CNT, the viscosity of the composite material even at high temperatures is increased such that the composite material may be processed by powder extrusion or flow pressing. Also, the powder can be directly processed by continuous powder rolling.

It is a remarkable advantage of the composite material of the invention that the beneficial mechanical properties of the powder particles can be maintained in the compacted finished or semi-finished article. For example, when using multi-scroll CNT and Al5xxx, by employing a mechanical alloying process as described in section 4 above, a composite material having a Vickers hardness of more than 390 HV was obtained. Remarkably, even after compacting the powder material to a finished connection means, the Vickers hardness remains at more than 80% of this value. In other words, due to the stabilizing nano structure, the hardness of the individual composite powder particles can largely be transferred to the compacted connection means. Prior to this invention, such a hardness in the compacted article was not possible.

### 6. MATERIAL CONNECTION

Fig. 13 shows a material connection 52 comprising a first part 54, a second part 56 and a connection means 58 connecting the first and second parts. For example, the first part 54 could be a portion of an engine block and the second part 56 could be a part of a cylinder head, which are attached to each other by the connection means 58 according to an embodiment of the invention. In such an application, the ideal connection means would have a high mechanical strength, a high thermal stability and a light weight. Unfortunately, as mentioned above, prior art light metal alloys such as high strength Al-alloys will have a small weight and a high mechanical strength, but fail to provide for thermal stability. Also, the manufacturing of connection means from such high strength aluminum alloys is difficult and costly for the reasons given above. In addition, even if a suitable metal alloy is found which has the desired mechanical properties, there is a further problem that the electrochemical potentials between the connection means and each of the first and second parts would be different, which would lead to a contact corrosion in the presence of a suitable electrolyte.

However, in the material connection 52 of Fig. 13, a connection means 58 according to an embodiment of the invention is used, which allows to control the mechanical properties of the connection means 58 by the content of nanoparticles, in particular CNT, rather than by the metal part used. Accordingly, the material connection 52 can be made by using the same metal components in each of the first and second parts 54, 56 and the connection means 58, where the desired mechanical properties of the connection means 58 are provided by the nanoparticle content based on the above nano-stabilization effect, such that no galvanic potential difference between the parts 54, 56 and the connection means 58 exists. This way, contact corrosion can be reliably prevented without compromising the mechanical properties of the connection means 58.

In practice, it is not necessary that all the metal components involved in the material connection 52 are identical, as long the difference in electrochemical potentials is low enough such as to prevent contact corrosion during the intended use. In many cases, contact corrosion can be avoided if the difference in chemical potential is less than 50 mV, preferably 25 mV.

Further, if the first part 54 would be a portion of an engine block and the second 56 would be a portion of the cylinder head, a suitable light weight material for forming the same would be A15xxx. In this case, the connection means 58, i.e. a connecting screw could be made by a compound material comprising the same metal content but with a fraction of 2 to 6wt% of CNT, which would provide the desired tensile strength. What is more, due to the nano-stabilization effect described above, the connection means 58 would also have a sufficient thermal stability such that the mechanical properties would be conserved even during extended operation in a high temperature environment. In fact, the increased thermal stability makes the connection means according to the invention well suitable for applications in engines, turbines or other applications where high temperatures arise. Further useful applications for the connection means of the invention in material connections are ultralight constructions, high-end sporting goods, aviation and aerospace technology and walking aids.

As has been explained with reference to Fig. 13, in the framework of the present invention, the mechanical properties of the connection means can be controlled via the content of nanoparticles, in particular CNT, rather than by the metal component used. This concept is not only applicable to the connection means 58, but also to the parts 54 and 56 connected thereby. To illustrate this, reference is made to Fig. 14, showing four parts 60a to 60d, each of which being comprised of a compound material of a metal reinforced by nanoparticles. In the embodiment shown in Fig. 14, it is assumed that the metal or metal alloy component of each of parts 60a to 60d is identical, but that the concentrations of nanoparticles, in particular CNT varies between the parts, as is schematically indicated by different densities of the dots in Fig. 14. Also, neighbouring parts 60a to 60d are connected with connection means 62 which are also made from the compound material of a metal reinforced by nanoparticles.

Even if the same metal component is used in each of parts 60a to 60d and the connection means, the mechanical properties of each of these elements can be controlled by a suitable content of nanoparticles. In particular, this means that a joint product 64 formed by the individual parts 60a to 60d will have different mechanical properties in different regions thereof. For example, the Vickers hardness and tensile strength of the left most part of joint product 64 constituted by part 60a will be larger than that of the rightmost end constituted by part 60d, due to a higher nanoparticle content. This way, a joint product can be formed from the same metal, having different nanoparticle contents and accordingly different mechanical properties in different regions. An exemplary application of this would for example be the wing of an airplane, where it would be desirable if the tensile strength of the wing material would be higher close to the fuselage than at the wing tips. Again, it is a great practical advantage that the same metal can be used in different regions of the joint product 46 and its connection means 62 and still each component 60a to 60d, 62 has mechanical properties that can be specifically adapted to its function. In particular, since the same metal components are used, contact corrosion problems can be avoided which would generally occur if metals or alloys with different chemical potentials were combined.

While it appears especially attractive to use the same metal component throughout each of the parts 60a to 60d and the connection means 62, the embodiment is not limited to this case. For practical purposes it would be sufficient if the metal components would be selected such that the electrochemical potentials of each two contacting components 60a to 60d, 62 would deviate by less than 50 mV, preferably less than 25 mV.

The same concept can be carried even one step further, in that different mechanical properties can be achieved in different regions of a single integral product 66 by locally varying the nanoparticle content, as is shown in Fig. 15. The integral part 66 is again formed by a metal or metal alloy reinforced by nanoparticles, where the concentration of nanoparticles differs in different regions of the integral part 66. In particular, as is schematically indicated by the density of dots, the concentration of nanoparticles on the left end of integral part 66 of Fig. 15 is higher than on the right end, which leads to a higher tensile strength and Vickers hardness on the left end of integral component 66.

Note that all materials, material combinations and manufacturing methods described above with specific reference to connection means may equally be applied for manufacturing the integral component 66 of Fig. 15. In particular, the same small crystallite sizes for causing nano stabilization may apply for the material of integral component 66 and preferably, the same type of CNT may be used. Also, the same manufacturing method based on producing a composite powder material and compacting the same into a finished integral part 66 may be applied.

With specific reference to the example of Fig. 15, it is noted that the integral part could very efficiently be produced by powder extrusion or powder rolling, where the nanoparticle compound is varied during rolling or extrusion. This could for example be achieved by preparing two or more different types of composite powder materials having different nanoparticle contents, possibly even a powder containing no nanoparticles at all, and appropriately mixing the composite powder materials on rolling or extrusion.

Moreover, the integral part 66 shown in Fig. 15 could also be manufactured by hot isostatic pressing, cold isostatic pressing or sintering of a powder material which has been arranged such that different concentrations of nanoparticles at different parts are present, as desired.

### Reference Signs

- 10: catalytic CVD apparatus
- 12: fluidized bed reactor
- 14: heating means
- 16: lower entrance
- 18: upper discharge opening
- 20: catalyst entrance
- 22: discharge opening
- 24: setup for generating a metal powder through atomization
- 26: vessel
- 28: heating means
- 30: chamber
- 32: argon driving gas
- 34: nozzle assembly
- 36: chamber
- 38: argon quenching gas
- 40: metal powder
- 42: high energy mill
- 44: milling chamber
- 46: rotating element
- 48: arm of rotating element 46
- 50: milling ball
- 52: material connection
- 54: first part
- 56: second part
- 58: connection means
- 60a - 60d: parts made from compound material
- 62: connection means
- 64: joint product
- 66: integral part

## Claims

1. A connection means (58) made from metal, and in particular Al, Mg, Cu or Ti, or an alloy comprising one or more thereof and in the form of a screw, a bracket, a hinge or a rivet, **characterized in that** the connection means (58) is made from a compound material of said metal reinforced by nanoparticles, in particulary carbon nanotubes (CNT), wherein the reinforced metal has a microstructure comprising metal crystallites at least partly separated by said nanoparticles.

2. The connection means (58) of claim 1, wherein a compound comprises metal crystallites having a size in a range of 1 nm to 100 nm, preferably 10 nm to 100 nm, or in a range of more than 100 nm and up to 200 nm.

3. The connection means (58) of one of the previous claims, wherein nanoparticles are also contained in at least some of the crystallites.

4. The connection means (58) of one of the previous claims, wherein the CNT content of the composite material by weight is in the range of 0.5 to 10.0%, preferably 2.0 to 9.0% and most preferably 3.0 to 6.0%.

5. The connection means (58) of one of the previous claims, wherein the nano particles are formed by CNTs, at least a fraction of which having a scroll structure comprised of one or more rolled up graphite layers, each graphite layer consisting of two or more graphene layers on top of each other.

6. The connection means (58) of one of the previous claims, wherein at least a fraction of the nano particles are functionalized, in particular roughened on their outer surface.

7. The connection means (58) of one of the previous claims, wherein the Vickers hardness of the compound material exceeds the Vickers hardness of the original metal by 40% or more, preferably by 80% or more.

8. The connection means (58) of one of the previous claims, wherein the metal is formed by an Al alloy and the Vickers hardness of the compound material is higher than 250 HV, preferably higher than 300 HV.

9. A material connection (52) comprising a first part (54), a second part (56) and a connection means (58) according to one of claims I to 8 connecting the first and second parts (54, 56), wherein at least one of the first and second parts (54, 56) comprises a metal or a metal alloy, and
wherein the connections means (58) is made from a compound material of a metal reinforced by nanoparticles,
wherein said metal or metal alloy of said at least one of said first and second parts (54, 56) is the same as that of the metal component of the connection means (58) or has an electrochemical potential deviating from that of the metal component of the connection means (58) by less than 50 mV, preferably, less than 25 mV.

10. The material connection (52) of claim 9, wherein at least two members of the group consisting of the first part (54), the second part (56) and the connection means (58) are made from a compound material of a metal or metal alloy reinforced by nanoparticles but have different concentrations of nanoparticles.

11. The material connection (58) of claim 10, wherein the numerical values of the percentage of nanoparticles by weight of said two members differ at least by 10%, preferably by at least 20% of the higher one of said numerical values.

12. The connection means (58) of one of claims 1 to 8, wherein the concentration of nanoparticles varies between different regions of said integral part.

13. The connection means (58) of claim 12, wherein the nanoparticle concentration varies along at least one direction of said integral part.

14. A method of manufacturing a connection means (58) in the form of a screw, a bracket, a hinge or a rivet, comprising the following steps:
producing a composite powder material, said material comprising a metal and nanoparticles, in particular carbon nano tubes (CNT),
said compound powder particles comprising metal crystallites at least partly separated from each other by said nano particles, and
a step of compacting the composite powder into a finished connection means (58).

15. The method of claim 14, wherein the step of compacting the composite powder comprises hot isostatic pressing cold isostatic pressing, powder extrusion, powder rolling, or sintering.

16. The method of claim 14 or 15, wherein the compound powder particles comprise light metal crystallites having a size in a range of 1 nm to 100 nm, preferably 10 nm to 100 nm, or in a range of more than 100 nm and up to 200 nm.

17. The method of one of claims 14 to 16, further comprising a step of processing a metal powder and said nano particles by mechanical alloying such as to form said compound powder.

18. The method of claim 17, wherein the metal powder and the nanoparticles are processed such that nanoparticles are also contained in at least some of the crystallites.

19. The method of one of claims 14 to 17, wherein said metal is a light metal, in particular Al, Mg, Ti or an alloy including one or more of the same, Cu or a Cu alloy.

20. The method of one of claims 14 to 19 , wherein said nano particles are formed by carbon nano tubes (CNT) provided in form of a powder of tangled CNT agglomerates having a mean size sufficiently large to allow easy handling because of a low potential for dustiness.

21. The method of claim 20, wherein at least 95% of the CNT agglomerates have a particle size larger than 100 µm.

22. The method of claims 20 or 21, wherein the mean diameter of the CNT agglomerates is between 0.05 and 5 mm, preferably between 0-1 and 2 mm and most preferably between 02 and I mm.

23. The method of one of claims 14 to 22, wherein the length to diameter ratio of the nano particles, in particular CNTs, is larger than 3, preferably larger than 10 and most preferably larger than 30.

24. The method of one of claims 14 to 23, wherein the CNT content of the composite material by weight is in a range of 0.5 to 10.0%, preferably 2.0 to 9.0% and most preferably 3.0 to 6.0%.

25. The method of one of claims 14 to 24, wherein the nano particles are formed by CNTs, at least a fraction of which having a scrolled structure, comprised of one or more rolled up graphite layers, each graphite layer consisting of two or more graphene layers on top of each other.

26. The method of one of claims 14 to 25, comprising a step of functionalizing, in particular roughening at least a fraction of the nano particles prior to the mechanical alloying.

27. The method of claim 26, wherein the nano particles are formed by multi-wall or multi-scroll CNTs and the roughening is performed by causing at least the outermost layer of at least some of the CNTs to break by submitting the CNTs to high pressure, in particular, a pressure of 5 MPa or higher, preferably 7.8 MPa or higher.

28. The method of one of claims 14 to 27, wherein the processing is conducted such as to increase and stabilize the dislocation density of the crystallites by the nanoparticles sufficiently to increase the average Vickers hardness of the composite material and/or of the connection means (58) formed by compacting the same to exceed the Vickers hardness of the original metal by 40% or more, preferably by 80% or more.

29. The method of one of claims 14 to 27, wherein the processing is conducted such as to stabilize the dislocations and suppress grain growth sufficiently such that the Vickers hardness of the connection means (58) formed by compacting the composite powder is higher than the Vickers hardness of the original metal, preferably higher than 80% of the Vickers hardness of the composite powder.

30. The method of one of claims 17 to 29, wherein the mechanical alloying is performed using a ball mill (42) comprising a milling chamber (44) and balls (50) as milling members.

31. The method of claim 30, wherein the balls (50) are accelerated to a speed of at least 5 m/s, preferably at least 8 m/s and most preferably at least 11 m/s.

32. The method of claim 30 or 31, wherein the milling chamber (44) is stationary and the balls (50) are accelerated by a rotary motion of a rotating element (46).

33. The method of claim 32, wherein an axis ofsaid rotating element (46) is oriented horizontally.

34. The method of one of claims 30 to 33, wherein said balls (50) have a diameter of 3 to 8 mm, preferably 3 to 6 mm and/or are made from steel, ZiO₂ or yttria stabilized ZrO₂.

35. The method of one of claims 30 to 34, wherein the volume *V_{b}* occupied by the balls (50) corresponds to *V_{b}* = *V_{c}* - π · (r*_{R}*)² · *l* ± 20%, wherein
*V_{c}* is the volume of the milling chamber (44), *r_{R}* is the radius of the rotating element (46) and *l* is the length of the milling chamber (44) in axial direction of the rotating element (46).

36. The method of one of claims 30 to 35, wherein an inert gas, in particular Ar, He or N₂ or a vacuum environment is provided inside the milling chamber (44).

37. The method of one of claims 30 to 36, wherein the ratio of (metal + nano particles)-to-balls by weight is between 1:7 and 1:13.

38. The method of one of claims 14 to 37, wherein said processing of metal powder and nano particles comprises a first and a second processing stage,
wherein in the first processing stage, most or all of the metal is processed, and
in the second stage, nano particles, in particular CNTs are added and the metal and the nano particles are simultaneously processed.

39. The method of claim 38, wherein a fraction of the nano particles is already added in the first processing stage to avoid sticking of the metal.

40. The method of one of claims 38 and 39, wherein the first stage is conducted for a time suitable to generate metal crystallites having an average size below 200 nm, preferably below 100 nm, and in particular for 20 to 60 min.

41. The method of one of claims 38 to 40, wherein the second stage is conducted for a time sufficient to cause a stabilization of the micro structure of the crystallites by the nano particles, and in particular for 5 to 30 min.

42. The method of one of claims 38 to 41, wherein the second stage is shorter than the first stage.

43. The method of one of claims 32 to 42, wherein during the processing, the rotational speed of the rotating element (46) is cyclically raised and lowered.

44. The method of one of claims 14 to 43, wherein said nano particles are formed by CNTs provided in the form of a CNT powder, said method further comprising a step of producing said CNT powder by catalytic carbon vapour deposition using one or more of a group consisting of acetylene, methane, ethane, ethylene, butane, butene, butadiene, and benzene as a carbon donor.

45. The method claim 44, wherein the catalyst comprises two or more elements of a group consisting of Fe, Co, Mn, Mo and Ni.

46. The method of one of claims 44 and 45, wherein said step of producing the CNT powder comprises a step of catalytic decomposition of C₁-C₃-carbohydrogens at 500°C to 1000°C using a catalyst comprising Mn and Co in a molaric ratio in a range of 2:3 to 3:2.

47. The method of one of claims 14 to 46, further comprising a step of forming a metal powder as the metal constituent of the composite material by spray atomization of a liquid metal or alloy into an inert atmosphere.

48. The method of one of claims 14 to 47, further comprising a step of passivating the finished composite material.

49. The method of claim 48, wherein the composite material is loaded into a passivation chamber and stirred therein while oxygen is gradually added such as to oxidize the composite material.

## Patentansprüche

1. Verbindungsmittel (58), hergestellt aus Metall, und insbesondere aus Al, Mg, Cu oder Ti oder aus einer Legierung, die eines oder mehrere dieser Materialien umfasst, und in Form einer Schraube, einer Halterung eines Scharniers oder eines Niets, **dadurch gekennzeichnet, dass** das Verbindungsmittel (58) aus einem Verbundwerkstoff des Metalls besteht, das durch Nanopartikel, insbesondere Kohlenstoffnanoröhren (CNT), verstärkt ist, wobei das verstärkte Metall eine Mikrostruktur aufweist, die Metallkristallite umfasst, die zumindest teilweise durch die Nanopartikel getrennt sind.

2. Verbindungsmittel (58) nach Anspruch 1, wobei der Verbundwerkstoff Metallkristallite in einem Größenbereich von 1 nm bis 100 nm, vorzugsweise 10 nm bis 100 nm oder in einem Bereich von mehr als 100 nm und bis zu 200 nm umfasst.

3. Verbindungsmittel (58) nach einem der vorstehend aufgeführten Ansprüche, wobei Nanopartikel auch in mindestens einigen der Kristallite enthalten sind.

4. Verbindungsmittel (58) nach einem der vorstehend aufgeführten Ansprüche, wobei der CNT-Gewichtsgehalt des Verbundwerkstoffs im Bereich von 0,5 bis 10,0%, vorzugsweise 2,0 bis 9,0% und besonders bevorzugt im Bereich von 3,0 bis 6,0% liegt.

5. Verbindungsmittel (58) nach einem der vorstehend aufgeführten Ansprüche, wobei die Nanopartikel durch CNTs gebildet sind, von denen mindestens ein Anteil eine Rollenstruktur aufweist, die aus einer oder mehreren aufgerollten Graphitschichten zusammengesetzt ist, wobei jede Graphitschicht aus zwei oder mehreren übereinanderliegenden Graphenschichten besteht.

6. Verbindungsmittel (58) nach einem der vorstehend aufgeführten Ansprüche, wobei mindestens ein Anteil der Nanopartikel funktionalisiert und insbesondere an ihrer Außenfläche aufgeraut ist.

7. Verbindungsmittel (58) nach einem der vorstehend aufgeführten Ansprüche, wobei die Vickershärte des Verbundwerkstoffs die Vickershärte des ursprünglichen Metalls um 40% oder mehr, vorzugsweise um 80% oder mehr übersteigt.

8. Verbindungsmittel (58) nach einem der vorstehend aufgeführten Ansprüche, wobei das Metall durch eine Al-Legierung gebildet ist und die Vickershärte des Verbundwerkstoffs mehr als 250 HV, vorzugsweise mehr als 300 HV beträgt.

9. Materialverbindung (52), die ein erstes Teil (54), ein zweites Teil (56) und ein Verbindungsmittel (58) nach einem der Ansprüche 1 bis 8 umfasst, das das erste und das zweite Teil (54, 56) miteinander verbindet, wobei das erste und/oder das zweite Teil (54, 56) ein Metall oder eine Metalllegierung umfasst, und
wobei das Verbindungsmittel (58) aus einem Verbundwerkstoff eines durch Nanopartikel verstärkten Metalls besteht, wobei das Metall oder die Metalllegierung des ersten und/oder des zweiten Teils (54, 56) mit demjenigen bzw. derjenigen der Metallkomponente des Verbindungsmittels (58) identisch ist oder ein elektrochemisches Potenzial hat, das von demjenigen der Metallkomponente des Verbindungsmittels (58) um weniger als 50 mV, vorzugsweise um weniger als 25 mV abweicht.

10. Materialverbindung (52) nach Anspruch 9, wobei mindestens zwei Elemente der Gruppe, die aus dem ersten Teil (54), dem zweiten Teil (56) und dem Verbindungsmittel (58) besteht, aus einem Verbundwerkstoff eines Metalls oder einer Metalllegierung, verstärkt durch Nanopartikel, bestehen, aber unterschiedliche Konzentrationen von Nanopartikeln aufweisen.

11. Materialverbindung (52) nach Anspruch 10, wobei die Zahlenwerte der Nanopartikel-Gewichtsanteile der zwei Elemente um mindestens 10%, bevorzugt um mindestens 20% des höheren der Zahlenwerte differieren.

12. Verbindungsmittel (58) nach einem der Ansprüche 1 bis 8, wobei die Konzentration von Nanopartikeln zwischen verschiedenen Bereichen des integralen Teils variiert.

13. Verbindungsmittel (58) nach Anspruch 12, wobei die Nanopartikelkonzentration entlang mindestens einer Richtung des integralen Teils variiert.

14. Verfahren zur Herstellung eines Verbindungsmittels (58) in Form einer Schraube, einer Halterung, eines Scharniers oder eines Niets, wobei das Verfahren die folgenden Schritte umfasst:
Herstellen eines Verbundpulverwerkstoffs, wobei der Werkstoff ein Metall und Nanopartikel, insbesondere Kohlenstoffnanoröhren (CNTs) umfasst,
wobei die Verbundpulverpartikel Metallkristallite umfassen, die zumindest teilweise durch die Nanopartikel voneinander getrennt sind, und
einen Schritt des Verdichtens des Verbundpulvers zu einem fertigen Verbindungsmittel (58).

15. Verfahren nach Anspruch 14, wobei der Schritt des Verdichtens des Verbundpulvers heißisostatisches Pressen, kaltisostatisches Pressen, Pulverstrangpressen, Pulverwalzen oder Sintern umfasst.

16. Verfahren nach Anspruch 14 oder 15, wobei die Verbundpulverpartikel Leichtmetallkristallite im Größenbereich von 1 nm bis 100 nm, vorzugsweise 10 nm bis 100 nm oder in einem Bereich von mehr als 100 nm und bis zu 200 nm umfassen.

17. Verfahren nach einem der Ansprüche 14 bis 16, das weiterhin einen Schritt des Verarbeitens eines Metallpulvers und der Nanopartikel durch mechanisches Legieren zur Bildung des Verbundpulvers umfasst.

18. Verfahren nach Anspruch 17, wobei das Metallpulver und die Nanopartikel so verarbeitet werden, dass die Nanopartikel auch in mindestens einigen der Kristallite enthalten sind.

19. Verfahren nach einem der Ansprüche 14 bis 17, wobei das Metall ein Leichtmetall, insbesondere Al, Mg, Ti oder eine Legierung, die eines oder mehrere dieser Materialien enthält, Cu oder eine Cu-Legierung ist.

20. Verfahren nach einem der Ansprüche 14 bis 19, wobei die Nanopartikel durch Kohlenstoffnanoröhren (CNT) hergestellt werden, die in Form eines Pulvers aus verknäulten CNT-Agglomeraten mit einer mittleren Größe, die groß genug ist, eine leichte Handhabung durch ein geringes Verstaubungspotenzial zu gestatten, vorgesehen sind.

21. Verfahren nach Anspruch 20, wobei mindestens 95% der CNT-Agglomerate eine Partikelgröße von über 100 µm aufweisen.

22. Verfahren nach Anspruch 20 oder 21, wobei der mittlere Durchmesser der CNT-Agglomerate zwischen 0,05 und 5 mm, vorzugsweise zwischen 0,1 und 2 mm und besonders bevorzugt zwischen 0,2 und 1 mm liegt.

23. Verfahren nach einem der Ansprüche 14 bis 22, wobei das Längen/Durchmesser-Verhältnis der Nanopartikel, insbesondere der CNTs, größer als 3, vorzugsweise grö-βer als 10 und besonders bevorzugt größer als 30 ist.

24. Verfahren nach einem der Ansprüche 14 bis 23, wobei der CNT-Gewichtsgehalt des Verbundwerkstoffs in einem Bereich von 0,5 bis 10,0%, vorzugsweise von 2,0 bis 9,0% und besonders bevorzugt von 3,0 bis 6,0% liegt.

25. Verfahren nach einem der Ansprüche 14 bis 24, wobei die Nanopartikel durch CNTs gebildet sind, wobei mindestens ein Anteil davon eine Rollenstruktur hat, die aus einer oder mehreren aufgerollten Graphitschichten besteht, wobei jede Graphitschicht aus zwei oder mehreren übereinanderliegenden Graphenschichten zusammengesetzt ist.

26. Verfahren nach einem der Ansprüche 14 bis 25, das einen Schritt des Funktionalisierens, insbesondere des Aufrauens von mindestens einem Anteil der Nanopartikel vor dem mechanischen Legieren umfasst.

27. Verfahren nach Anspruch 26, wobei die Nanopartikel durch mehrwandige oder mehrfach aufgerollte CNTs gebildet sind und das Aufrauen dadurch erfolgt, dass bewirkt wird, dass mindestens die äußerste Schicht von mindestens einigen der CNTs aufgebrochen wird, indem die CNTs einem hohen Druck, insbesondere einem Druck von 5 MPa oder höher, vorzugsweise 7,8 MPa oder höher ausgesetzt werden.

28. Verfahren nach einem der Ansprüche 14 bis 27, wobei das Verarbeiten so durchgeführt wird, dass die Versetzungsdichte der Kristallite durch die Nanopartikel in ausreichendem Maße erhöht und stabilisiert wird, um die durchschnittliche Vickershärte des Verbundwerkstoffs und/oder des durch dessen Verdichtung gebildeten Verbindungsmittels (58) zu erhöhen, so dass die Vickershärte des ursprünglichen Metalls um 40% oder mehr, vorzugsweise um 80% oder mehr überschritten wird.

29. Verfahren nach einem der Ansprüche 14 bis 27, wobei das Verarbeiten so durchgeführt wird, dass die Versetzungen stabilisiert werden und das Kornwachstum in ausreichendem Maße unterdrückt wird, so dass die Vickershärte des durch Verdichtung des Verbundpulvers gebildeten Verbindungsmittels (58) höher als die Vickershärte des ursprünglichen Metalls, vorzugsweise höher als 80% der Vickershärte des Verbundpulvers ist.

30. Verfahren nach einem der Ansprüche 17 bis 29, wobei das mechanische Legieren unter Verwendung einer Kugelmühle (42) erfolgt, die eine Mahlkammer (44) und Kugeln (50) als Mahlelemente umfasst.

31. Verfahren nach Anspruch 30, wobei die Kugeln (50) auf eine Geschwindigkeit von mindestens 5 m/s, vorzugsweise auf mindestens 8 m/s und besonders bevorzugt auf mindestens 11 m/s beschleunigt werden.

32. Verfahren nach Anspruch 30 oder 31, wobei die Mahlkammer (44) stationär ist und die Kugeln (50) durch eine Drehbewegung eines rotierenden Elements (46) beschleunigt werden.

33. Verfahren nach Anspruch 32, wobei eine Achse des rotierenden Elements (46) horizontal angeordnet ist.

34. Verfahren nach einem der Ansprüche 30 bis 33, wobei die Kugeln (50) einen Durchmesser von 3 bis 8 mm, vorzugsweise von 3 bis 6 mm haben und/oder aus Stahl, ZiO₂ oder aus yttriumoxidstabilisiertem ZiO₂ bestehen.

35. Verfahren nach einem der Ansprüche 30 bis 34, wobei das Volumen V_{b}, das von den Kugeln (50) eingenommen wird, V_{b} = V_{c} - π · (r_{R})² · l ± 20% entspricht, wobei V_{c} das Volumen der Mahlkammer (44), r_{R} der Radius des rotierenden Elements (46) und 1 die Länge der Mahlkammer (44) in axialer Richtung des rotierenden Elements (46) ist.

36. Verfahren nach einem der Ansprüche 30 bis 34, wobei ein Inertgas, insbesondere Ar, He oder N₂, oder eine Vakuumumgebung im Inneren der Mahlkammer (44) bereitgestellt wird.

37. Verfahren nach einem der Ansprüche 30 bis 36, wobei das Gewichtsverhältnis (Metall + Nanopartikel)/ Kugeln zwischen 1:7 und 1:13 liegt.

38. Verfahren nach einem der Ansprüche 14 bis 37, wobei das Verarbeiten von Metallpulver und Nanopartikeln eine erste und eine zweite Verarbeitungsstufe umfasst, wobei in der ersten Verarbeitungsstufe das meiste oder das gesamte Metall verarbeitet wird, und wobei in der zweiten Stufe Nanopartikel, insbesondere CNTs, hinzugefügt und das Metall und die Nanopartikel gleichzeitig verarbeitet werden.

39. Verfahren nach Anspruch 38, wobei ein Anteil der Nanopartikel bereits in der ersten Verarbeitungsstufe hinzugefügt werden, um ein Verkleben des Metalls zu verhindern.

40. Verfahren nach einem der Ansprüche 38 und 39, wobei die erste Stufe über eine Zeitdauer durchgeführt wird, die geeignet ist, Metallkristallite mit einer durchschnittlichen Größe von weniger als 200 nm, bevorzugt weniger als 100 nm, zu erzeugen, und wobei die Zeitdauer insbesondere 20 bis 60 Min. beträgt.

41. Verfahren nach einem der Ansprüche 38 bis 40, wobei die zweite Stufe über eine Zeitdauer durchgeführt wird, die ausreicht, um eine Stabilisierung der Mikrostruktur der Kristallite durch die Nanopartikel zu bewirken, und wobei die Zeitdauer insbesondere 5 bis 30 Min. beträgt.

42. Verfahren nach einem der Ansprüche 38 bis 41, wobei die zweite Stufe kürzer als die erste Stufe ist.

43. Verfahren nach einem der Ansprüche 32 bis 42, wobei während des Verarbeitens die Drehgeschwindigkeit des rotierenden Elements (46) zyklisch gesteigert und abgesenkt wird.

44. Verfahren nach einem der Ansprüche 14 bis 43, wobei die Nanopartikel durch CNTs gebildet werden, die in der Form eines CNT-Pulvers bereitgestellt werden, und wobei das Verfahren weiterhin einen Schritt des Herstellens des CNT-Pulvers durch katalytische Kohlenstoffaufdampfung unter Verwendung von einem oder mehreren Materialien aus einer Gruppe umfasst, zu der Acetylen, Methan, Ethan, Ethylen, Butan, Buten, Butadien und Benzol als Kohlenstoffspender zählen.

45. Verfahren nach Anspruch 44, wobei der Katalysator zwei oder mehrere Elemente aus einer Gruppe umfasst, zu der Fe, Co, Mn, Mo und Ni zählen.

46. Verfahren nach einem der Ansprüche 44 und 45, wobei der Schritt des Herstellens des CNT-Pulvers einen Schritt des katalytischen Zersetzens von C₁-C₃-Carbohydrogenen bei 500°C bis 1000°C unter Verwendung eines Katalysators umfasst, der Mn und Co in einem Molverhältnis in einem Bereich von 2:3 bis 3:2 umfasst.

47. Verfahren nach einem der Ansprüche 14 bis 46, wobei das Verfahren weiterhin einen Schritt des Bildens eines Metallpulvers als Metallbestandteil des Verbundwerkstoffs durch Sprühzerstäubung eines Flüssigmetalls oder einer Flüssiglegierung in einer inerten Atmosphäre umfasst.

48. Verfahren nach einem der Ansprüche 14 bis 47, wobei das Verfahren weiterhin einen Schritt des Passivierens des fertigen Verbundwerkstoffs umfasst.

49. Verfahren nach Anspruch 48, wobei der Verbundwerkstoff in eine Passivierungskammer eingebracht und darin umgerührt wird, während Sauerstoff nach und nach zugegeben wird, um so den Verbundwerkstoff zu oxidieren.

## Revendications

1. Moyen de connexion (58) constitué de métal, et en particulier d'Al, Mg, Cu ou Ti, ou d'un alliage comprenant un ou plusieurs de ces éléments et sous la forme d'une vis, d'une fixation, d'une charnière ou d'un rivet, **caractérisé en ce que** le moyen de connexion (58) est constitué d'un matériau composite composé dudit métal renforcé par des nano-particules, en particulier des nano-tubes de carbone (CNT), le métal renforcé présentant une micro-structure comprenant des cristallites de métal qui sont au moins partiellement séparées par lesdites nano-particules.

2. Moyen de connexion (58) selon la revendication 1, dans lequel un composite comprend des cristallites de métal dont la taille est comprise dans une gamme de 1 nm à 100 nm, de préférence de 10 nm à 100 nm, ou dans une gamme de plus de 100 nm et jusqu'à 200 nm.

3. Moyen de connexion (58) selon l'une des revendications précédentes, dans lequel des nano-particules sont également contenues dans au moins plusieurs des cristallites.

4. Moyen de connexion (58) selon l'une des revendications précédentes, dans lequel la teneur en CNT du matériau composite en poids se situe dans la gamme de 0,5 % à 10,0 %, de préférence de 2,0 % à 9,0 %, et idéalement de 3,0 % à 6,0 %.

5. Moyen de connexion (58) selon l'une des revendications précédentes, dans lequel les nano-particules sont formées par des CNT, dont au moins une fraction présente une structure de volute qui est constituée d'une ou de plusieurs couche(s) de graphite enroulée(s), chaque couche de graphite étant constituée de deux ou plus de deux couches de graphène les unes au-dessus des autres.

6. Moyen de connexion (58) selon l'une des revendications précédentes, dans lequel au moins une fraction des nano-particules sont fonctionnalisées, en particulier rendues rugueuses sur leur surface extérieure.

7. Moyen de connexion (58) selon l'une des revendications précédentes, dans lequel la dureté Vickers du matériau composite dépasse la dureté Vickers du métal original de 40 % ou plus, de préférence de 80 % ou plus.

8. Moyen de connexion (58) selon l'une des revendications précédentes, dans lequel le métal est constitué par un alliage d'Al, et la dureté Vickers du matériau composite est supérieure à 250 HV, de préférence supérieure à 300 HV.

9. Connexion de matériau (52) comprenant une première partie (54), une deuxième partie (56) et un moyen de connexion (58) selon l'une des revendications 1 à 8 qui relie les première et deuxième parties (54, 56), dans laquelle au moins une des première et deuxième parties (54, 56) comprend un métal ou un alliage de métal, le moyen de connexion (58) étant constitué d'un matériau composite composé d'un métal renforcé par des nano-particules, ledit métal ou alliage de métal de ladite au moins une desdites première et deuxième parties (54, 56) étant le même que celui du composant de métal du moyen de connexion (58) ou présentant un potentiel électrochimique qui s'écarte de celui du composant de métal du moyen de connexion (58) de moins de 50 mV, de préférence de moins de 25 mV.

10. Connexion de matériau (52) selon la revendication 9, dans laquelle au moins deux éléments du groupe comprenant la première partie (54), la deuxième partie (56) et le moyen de connexion (58) sont constitués d'un matériau composite composé d'un métal ou d'un alliage de métal renforcé par des nano-particules mais présentent des concentrations différentes de nano-particules.

11. Connexion de matériau (52) selon la revendication 10, dans laquelle les valeurs numériques du pourcentage de nano-particules en poids desdits deux éléments diffèrent d'au moins 10 %, de préférence d'au moins 20 % de la plus élevée desdites valeurs numériques.

12. Moyen de connexion (58) selon l'une quelconque des revendications 1 à 8, dans lequel la concentration de nano-particules varie entre différentes régions de ladite partie intégrale.

13. Moyen de connexion (58) selon la revendication 12, dans lequel la concentration de nano-particules varie le long d'au moins une direction de ladite partie intégrale.

14. Procédé de fabrication d'un moyen de connexion (58) sous la forme d'une vis, d'une fixation, d'une charnière ou d'un rivet, comprenant les étapes suivantes:
un matériau de poudre composite, ledit matériau comprenant un métal et des nano-particules, en particulier des nano-tubes de carbone (CNT),
lesdites particules de poudre composite comprenant des cristallites de métal au moins partiellement séparées les unes des autres par lesdites nano-particules, et
une étape de compactage de la poudre composite en un moyen de connexion (58) fini.

15. Procédé selon la revendication 14, dans lequel l'étape de compactage de la poudre composite comprend un pressage isostatique à chaud, un pressage isostatique à froid, une extrusion de poudre, un laminage de poudre ou un frittage.

16. Procédé selon la revendication 14 ou 15, dans lequel les particules de poudre composite comprennent des cristallites de métal léger dont la taille est comprise dans une gamme de 1 nm à 100 nm, de préférence de 10 nm à 100 nm, ou dans une gamme de plus de 100 nm et jusqu'à 200 nm.

17. Procédé selon l'une des revendications 14 à 16, comprenant en outre une étape de traitement d'une poudre de métal et desdites nano-particules par alliage mécanique de manière à former ladite poudre composite.

18. Procédé selon la revendication 17, dans lequel la poudre de métal et les nano-particules sont traitées de telle sorte que des nano-particules soient également contenues dans au moins plusieurs des cristallites.

19. Procédé selon l'une des revendications 14 à 17, dans lequel ledit métal est un métal léger, en particulier Al, Mg ou Ti, ou un alliage comprenant un ou plusieurs de ces éléments, Cu ou un alliage de Cu.

20. Procédé selon l'une quelconque des revendications 14 à 19, dans lequel lesdites nano-particules sont formées par des nano-tubes de carbone (CNT) prévus sous forme d'une poudre d'agglomérés de CNT entremêlés ayant une taille moyenne suffisamment grande pour permettre une manipulation aisée en raison d'une faible formation potentielle de poussière.

21. Procédé selon la revendication 20, dans lequel au moins 95 % des agglomérés de CNT ont une taille de particule supérieure à 100 µm.

22. Procédé selon la revendication 20 ou 21, dans lequel le diamètre moyen des agglomérés de CNT est compris entre 0,05 mm et 5 mm, de préférence entre 0,1 mm et 2 mm, et idéalement entre 0,2 mm et 1 mm.

23. Procédé selon l'une des revendications 14 à 22, dans lequel le rapport longueur - diamètre des nano-particules, en particulier des CNT, est supérieur à 3, de préférence supérieur à 10, et idéalement supérieur à 30.

24. Procédé selon l'une des revendications 14 à 23, dans lequel la teneur en CNT du matériau composite en poids se situe dans une gamme de 0,5 % à 10,0 %, de préférence de 2,0 % à 9,0 %, et idéalement de 3,0 % à 6,0 %.

25. Procédé selon l'une des revendications 14 à 24, dans lequel les nano-particules sont formées par des CNT, dont au moins une fraction présente une structure de volute qui est constituée d'une ou de plusieurs couche(s) de graphite enroulée(s), chaque couche de graphite étant constituée de deux ou plus de deux couches de graphène les unes au-dessus des autres.

26. Procédé selon l'une des revendications 14 à 25, comprenant une étape de fonctionnalisation, en particulier ayant pour but de la rendre rugueuse, d'au moins une fraction des nano-particules avant l'alliage mécanique.

27. Procédé selon la revendication 26, dans lequel les nano-particules sont formées par des CNT à parois multiples ou à volutes multiples, et l'étape consistant à rendre rugueux est exécutée en amenant au moins la couche extérieure extrême d'au moins une partie des CNT à se casser en soumettant les CNT à une pression élevée, en particulier une pression de 5 MPa ou plus, de préférence de 7,8 MPa ou plus.

28. Procédé selon l'une des revendications 14 à 27, dans lequel le traitement est conduit de manière à augmenter et à stabiliser la densité de dislocations des cristallites par les nano-particules suffisamment pour augmenter la dureté Vickers moyenne du matériau composite et/ou du moyen de connexion (58) qui est formé en compactant celui-ci de manière à dépasser la dureté Vickers du métal original de 40 % ou plus, de préférence de 80 % ou plus.

29. Procédé selon l'une des revendications 14 à 27, dans lequel le traitement est conduit de manière à stabiliser les dislocations et à supprimer le grossissement des grains suffisamment pour que la dureté Vickers du moyen de connexion (58) formé en compactant la poudre composite soit supérieure à la dureté Vickers du métal original, de préférence supérieure à 80 % de la dureté Vickers de la poudre composite.

30. Procédé selon l'une des revendications 17 à 29, dans lequel l'alliage mécanique est exécuté en utilisant un broyeur à billes (42) qui comprend une chambre de broyage (44) et des billes (50) comme éléments de broyage.

31. Procédé selon la revendication 30, dans lequel les billes (50) sont accélérées jusqu'à une vitesse d'au moins 5 m/s, de préférence d'au moins 8 m/s, et idéalement d'au moins 11 m/s.

32. Procédé selon la revendication 30 ou 31, dans lequel la chambre de broyage (44) est stationnaire, et les billes (50) sont accélérées par un mouvement de rotation d'un élément rotatif (46).

33. Procédé selon la revendication 32, dans lequel un axe dudit élément rotatif (46) est orienté horizontalement.

34. Procédé selon l'une des revendications 30 à 33, dans lequel lesdites billes (50) présentent un diamètre qui est compris entre 3 mm et 8 mm, de préférence entre 3 mm et 6 mm, et/ou sont constitués d'acier, de ZiO₂ ou de ZiO₂ stabilisé à l'oxyde d'yttrium.

35. Procédé selon l'une des revendications 30 à 34, dans lequel le volume V_{b} occupé par les billes (50) correspond à *V_{b}* = *V_{c}* - π · *(r*_{R}*)²* · *l* ± *20* %, où *V_{c}* est le volume de la chambre de broyage (44), *r_{R}* est le rayon de l'élément rotatif (46) et *l* est la longueur de la chambre de broyage (44) dans la direction axiale de l'élément rotatif (46).

36. Procédé selon l'une des revendications 30 à 35, dans lequel un gaz inerte, en particulier de l'Ar, de l'He ou du N₂ ou un environnement sous vide est prévu à l'intérieur de la chambre de broyage (44).

37. Procédé selon l'une des revendications 30 à 36, dans lequel le rapport du (métal plus les nano-particules) aux billes en poids est compris entre 1:7 et 1:13.

38. Procédé selon l'une des revendications 14 à 37, dans lequel ledit traitement de la poudre de métal et des nano-particules comprend une première et une deuxième étapes de traitement :
lors de la première étape de traitement, la majeure partie ou la totalité du métal est traité, et
lors de la deuxième étape, des nano-particules, en particulier des CNT, sont ajoutées et le métal et les nano-particules sont traités simultanément.

39. Procédé selon la revendication 38, dans lequel une fraction des nano-particules est déjà ajoutée lors de la première étape de traitement afin d'éviter le collage du métal.

40. Procédé selon l'une des revendications 38 et 39, dans lequel la première étape est conduite pendant une durée appropriée pour générer des cristallites de métal dont la taille moyenne est inférieure à 200 nm, de préférence inférieure à 100 nm, et en particulier pendant 20 à 60 minutes.

41. Procédé selon l'une des revendications 38 à 40, dans lequel la deuxième étape est conduite pendant une durée suffisante pour entraîner une stabilisation de la micro-structure des cristallites par les nano-particules, et en particulier pendant 5 à 30 minutes.

42. Procédé selon l'une des revendications 38 à 41, dans lequel la deuxième étape est plus courte que la première étape.

43. Procédé selon l'une des revendications 32 à 42, dans lequel, pendant le traitement, la vitesse de rotation de l'élément rotatif (46) est augmentée et réduite de façon cyclique.

44. Procédé selon l'une des revendications 14 à 43, dans lequel lesdites nano-particules sont formées par des CNT qui sont prévus sous la forme d'une poudre de CNT, ledit procédé comprenant en outre une étape de production de ladite poudre de CNT par dépôt catalytique de vapeur de carbone en utilisant un ou plusieurs éléments parmi un groupe comprenant l'acétylène, le méthane, l'éthane, l'éthylène, le butane, le butène, le butadiène et le benzène comme donneur de carbone.

45. Procédé selon la revendication 44, dans lequel le catalyseur comprend deux ou plus de deux éléments d'un groupe comprenant Fe, Co, Mn, Mo et Ni.

46. Procédé selon l'une des revendications 44 et 45, dans lequel ladite étape de production de la poudre de CNT comprend une étape de décomposition catalytique d'hydrocarbures C₁-C₃ réalisée entre 500°C et 1000°C en utilisant un catalyseur contenant du Mn et du Co en un rapport molaire qui est compris dans une gamme de 2:3 à 3:2.

47. Procédé selon l'une des revendications 14 à 46, comprenant en outre une étape de formation d'une poudre de métal comme composant métallique du matériau composite par pulvérisation d'un métal ou d'un alliage liquide dans une atmosphère inerte.

48. Procédé selon l'une des revendications 14 à 47, comprenant en outre une étape de passivation du matériau composite fini.

49. Procédé selon la revendication 48, dans lequel le matériau composite est chargé dans une chambre de passivation et est agité dans celle-ci pendant que de l'oxygène est progressivement ajouté de manière à oxyder le matériau composite.
